

## UNITED STATES PATENT OFFICE

JOSE MARTINEZ ESTAPE, OF HABANA, CUBA

## PROCESS OF PRODUCING PULP

No Drawing. Application filed April 5, 1928, Serial No. 267,806, and in Cuba January 18, 1928.

This invention relates to the use of plants heretofore never used for any industrial purpose and its object is to provide a new process of producing pulp from said plants.

In nearly all the climates of the world, and very specially, in the verges of brooks, rivers, everglades, etc., and in places where the soil contains some moisture, are born and grow, practically without cultivation, the plants called "carrizo", the scientific name of which is "*Arundo donax*" and her varieties, and the one called "reeds" the scientific name of which is "*Glycerium saccharoides*", all of these plants of the family of the gramineous or gramineous, and which are perfectly well known by their specific physic characteristics, such as smooth, hard and waterproof bark, with knots in their stems that form hollow internodes, brittle fibers, etc.

In the components of the reeds and the carrizo, there are, in its formation, celluloses in fibrous and ligneous condition, gums and mucilages which are soluble and insoluble, etc., and precisely, the cellulose extracted by means of my invention is specially adapted for the manufacture of paper, cardboard, artificial silk, gun cotton, etc., employing for the purpose some chemical and thermochemical components and special methods, which, when applied to the above named plants, produce the cellulose or pulp for the manufacture of all the articles mentioned and others which it would be obvious to enumerate here, all of which is bound to produce a real revolution in the textile and paper industries, due to the extremely low price at which the cellulose or pulp aforesaid may be sold due to the insignificant cost of the raw matter, because spreading the reeds or the carrizo once (in the places where there is none) it is not necessary to spread it again, but due to its nature and easy reproduction, the more it is cut, the stronger and more abundantly it sprouts, without the need of any subsequent cultivation.

The process for producing pulp from the "reed" or the "carrizo" plant, is as follows. The "reed" or the "carrizo" plant stalks are crushed in order to extract the juice which after fermenting is converted into alcohol,

and once crushed in small pieces to make it easier to handle, it is introduced into a boiler or special receptacle, with water at the rate of eight and half parts of water per one part of bagasse in weight, to which is added 8 to 9 percent of caustic soda, alone or with some small quantity of sodium sulphite, if the cellulose is to be employed in the manufacture of very fine paper or artificial silk. With this lye, the "reed" or the "carrizo" bagasse is boiled under a pressure of three to five atmospheres, during a period of half an hour to two hours, according to the kind of product to be made of the pulp, because on this depends the pressure and duration of the boiling period. The steam produced in the boiler is allowed to escape, and the lye is extracted, which, in being treated with hydrochloric acid gases, leave the gums contained by the bagasse separated from the pulp; these gums being applicable to many industries, and leaves the clarified liquid which is nothing more than sodium chloride, which serves for preparing the new lye for the new manufacturing process, thus greatly diminishing the cost and quantity of the soda, which is not needed then in the same proportion previously expressed.

The cellulose, paste or pulp remaining, is passed through a mill, in order to completely break up the fibre and reduce it to the size desired, according to the industry in which it is desired to use it, and then a perfect wash and sifting are carried out in order to take off the long fibres or the heavy threads which might have been left, which are passed again to the mill for further reduction.

The cellulose, paste or pulp remaining is already in a condition that permits its immediate introduction to a paper mill, for instance, where it may be entirely bleached with a solution of sodium hypochlorite of 3% and at a temperature of 40° C., or by means of the electrolytic chlorine, if the lyes resulting from the boiling are regenerated electrolytically upon taking them off the receptacle where the softening of the "reed" or the "carrizo" bagasse took place.

The cellulose thus extracted, due to its high grade of purity may be already em-

ployed for the manufacture of gun cotton or artificial silk or any other use where a cellulose, pulp or paste of the most pure and clean condition is required.

8 Having thus described my invention, what I claim is the following:—

1. A process for producing pulp from the "reed" (*Caña brava*) and the "carrizo" plants comprising, crushing the stalks of 10 said plants, boiling the resultant bagasse with water in the proportion of from 8½ to 10 parts of water to 1 part of bagasse by weight containing soda caustic and sodium sulphite in a receptacle under pressure treating the pulp with hydrochloric acid gas, separating from the pulp the gums contained in the bagasse, separating the liquor from the pulp, and crushing the separated pulp.
2. A process for producing pulp from the 20 "reed" (*Caña brava*) and the "carrizo" plants comprising, crushing the stalks of said plants, boiling the resultant bagasse with water containing soda caustic and sodium sulphite in a receptacle under pressure, 25 treating the pulp with hydrochloric acid gas, separating from the pulp the gums contained in the bagasse, separating the liquor from the pulp, crushing the separated pulp, washing and sifting it and crushing again the resulting fibers.

In witness whereof I affix my signature.

JOSE MARTINEZ ESTAPE.

35

40

45

50

55

60

65